

## UNITED STATES PATENT OFFICE

2,533,394

METHOD OF OBTAINING LARGE GRAIN  
SIZE IN SILICON STEEL

Everett W. Oppenheimer and Jack E. Lucas, Butler, Pa., assignors to Armco Steel Corporation, a corporation of Ohio

No Drawing. Application February 20, 1947,  
Serial No. 729,876

8 Claims. (Cl. 148—12.5)

1

Our invention has for its principal object the provision of an improved procedure for manufacturing silicon steel of good permeability and low core loss. It is applicable especially to the intermediate grades of silicon steel, which are produced under highly competitive conditions.

More specifically, our invention has as an object the attainment in a less expensive fashion of the combined features of low carbon content and large grain size, and the attainment of improved magnetic qualities in the material as compared with the best commercially economical procedures hitherto known.

It has long been understood that a large grain size could be obtained by a critical strain procedure applied to silicon steel of finished gauge. This, however, involves subjecting the cold-reduced material to an intermediate, strain-relieving anneal, followed by a carefully controlled "critical strain" in the nature of cold-work, preceding the final anneal. Such procedure is expensive, and the magnetic requirements for intermediate grades of silicon steel make it difficult to accomplish. For low production costs it is necessary that the intermediate grades of electrical steel be produced by a routing in which the cold reduced strip or sheet is given only a continuous or open anneal after it reaches finished gauge. One of the objects of the invention is to provide a routing which employs, after cold-reduction to gauge, a single heat treatment, but which nevertheless is productive of the improved results.

In a procedure outlined in Patent No. 2,358,788, a relatively large grain size and low carbon is attained in the final product by employing a phenomenon which may be termed "grain growth inheritance," i. e. a large grain size is attained in the hot-roller, intermediate gauge product as a result of straining the product and then box annealing it with the hot mill scale still on its surfaces. As a result of the attainment of this initial large grain size, after the subsequent cold-rolling to gauge and final open annealing, the grain size is found to be substantially and usefully larger than would otherwise be the case. The box annealing at around 1400° F. decarburizes the material by causing the oxidation of carbon and the concurrent reduction of the hot mill scale; and the large grain size of the intermediate product is attained during this anneal.

But this procedure involves carefully controlled cold work on the hot-rolled intermediate product, which is a matter of inconvenience and expense. Moreover, a type of scale which is quite

2

difficult to pickle away is left on the metal surfaces by the combination of the cold work on the scalped metal and the box anneal. Still other objects of this invention are the production of a large grain size in the final product without critical straining or other carefully controlled cold work at any stage of the routing, and an improvement of the scale conditions resulting from a decarburizing anneal.

10 These and other objects of our invention which will be set forth hereinafter or will be apparent to one skilled in the art upon reading these specifications, we accomplish by that procedure of which we will now describe an exemplary embodiment.

In our invention a simpler and less expensive method of producing the initial large grain size has been found, and its influence persists through the cold reductions and shows up as an equally 20 large or still larger grain size than that hitherto obtainable after the final open anneal. This, in turn, results in improved magnetic properties.

In the practice of our invention, we start with a ferrous material containing from about 1.00 25 to 3.50% silicon, depending on the magnetic properties required and subject it to the following routing:

1. The material is hot rolled to an intermediate gauge, say around .062 inch.
2. The hot-rolled product, with the hot mill scale still on its surfaces, is box annealed at around 1200° to 1700° (preferably 1400° F.).
3. It is then open annealed at from 1700° to 2100° F., and pickled.
4. It is next cold-rolled to the desired finished gauge.
5. Finally it is open annealed at 1700° to 2100° F.

The box anneal, which is step 2 of the routing, 40 is at the proper temperature for decarburization, and in this anneal the carbon will be reduced to around .015 or lower.

Unlike the method of Patent 2,358,788, we do not attain the desired large grain size in this 45 anneal for the reason that we omit the previous step of that patent in which the material was subjected to a carefully controlled amount of cold work.

We have discovered, however, that when the 50 carbon has been reduced in silicon steel to around .015 or lower, an open anneal at around 2000° F., which is step 3 of our routing, causes the material to anneal rapidly to an unusually uniform and large grain size, although the material 55 has not previously been strained by cold work.

The mechanism of this phenomenon is not fully explained. Apparently, the rapid attainment of the large grain size is the result of the coaction of the decarburizing anneal and the high temperature open anneal, and is a phenomenon occurring with material of low carbon content.

By an "open" anneal we mean a continuous or strand anneal in which the material is passed in a single thickness through an elongated furnace, the surfaces of the material being open or exposed to the furnace atmosphere, without limitation to the nature of the furnace atmosphere.

Since the material will be pickled immediately after the first open anneal (step 3) the nature of the furnace atmosphere during this step is unimportant. Ordinarily, we employ a furnace which is simply filled with the products of combustion of the heating fuel. The temperature of the open anneal should be varied with the silicon content for maximum grain size. Thus, for materials varying from 1% to 3½% silicon, the temperature of this open anneal may be varied from about 1700° F. for the lower silicon value to about 2100° F. for the higher silicon value.

Another result of the combination of steps thus far commented upon is that the scale remaining on the material after the initial open anneal is a scale which is readily pickled away, much more so than is the scale immediately following the box anneal, and especially where there has been previous cold work as in the process of Patent 2,358,788.

The final open anneal (step 5 of the process) is preferably carried on in a non-oxidizing or reducing atmosphere to avoid the necessity of a subsequent pickle. Here again the temperature of the anneal is advantageously varied in accordance with the silicon content of the steel as described above in connection with step 3.

When material treated in accordance with our process is pickled, cold reduced to the desired finished gauge, say .025-.014", and finally open annealed, the resulting grain size will be found to be sufficiently large to meet the requirements of the intermediate grades of silicon steel. This again is believed to be a phenomenon of grain growth inheritance. But our materials have improved magnetic properties as compared with products made by routings involving a small cold reduction ahead of the box anneal.

Modifications may be made in our invention without departing from the spirit of it. Having thus described our invention in an exemplary embodiment, what we claim as new and desire to secure by Letters Patent is:

1. A process of producing enhanced grain size in intermediate grade silicon steel which comprises subjecting hot rolled silicon steel to a box anneal at substantially from 1200° to 1700° F. with the hot mill scale still on its surfaces, to decarburize the steel to a carbon value not higher than substantially .015%, and then without intervening cold reduction, subjecting the steel to an open anneal at temperatures between substantially 1700° and 2100° F., preparatory to producing further reduction in the thickness of the steel.

2. The process claimed in claim 1, in which the temperature of the said open anneal is varied directly with the silicon content of the steel.

3. The process of claim 2 followed by a cold rolling and a final open anneal at substantially 1700° to 2100° F.

4. The process of claim 3 in which the temperature is varied directly with the silicon content.

5. A process of producing silicon steel of enhanced grain size and good magnetic properties which comprises subjecting hot rolled silicon steel at an intermediate gauge to a box anneal at substantially from 1200° to 1700° F. with the hot mill scale still on its surfaces, to decarburize the steel to a carbon content not substantially greater than .015%, subjecting the decarburized steel without intervening cold work to an open anneal at substantially 1700° to 2100° F. to produce a large grain size therein, then cold rolling the steel to final gauge, and developing the ultimate magnetic properties of the steel by an annealing treatment.

6. A process of producing silicon steel for magnetic uses which includes the successive steps of subjecting hot rolled silicon steel to a box anneal at substantially 1200° to 1700° F. while the hot mill scale remains on the surfaces of the steel whereby to decarburize it to a carbon value not substantially greater than .015%, and then without intervening treatment subjecting the steel to an open anneal at substantially 1700° to 2100° F. whereby to develop a large grain size therein and to convert any remaining scale on the steel surfaces to a condition in which it can readily be removed by pickling.

7. A process of producing silicon steel for magnetic uses which comprises hot rolling silicon steel containing substantially 1% to 3.5% silicon to an intermediate gauge, and without removing the hot mill scale, box annealing the silicon steel at a temperature of substantially 1200° to 1700° F., then without intervening treatment open annealing the steel at a temperature of substantially 1700° to 2100° F., then cold rolling the steel to finished gauge, and developing its ultimate magnetic properties by open annealing it at a temperature of substantially 1700° to 2100° F.

8. The process of claim 7 in which the temperature of both open anneals is varied directly with the silicon content of the steel.

EVERETT W. OPPENHEIMER.  
JACK E. LUCAS.

#### REFERENCES CITED

The following references are of record in the file of this patent:

#### UNITED STATES PATENTS

| 60 | Number    | Name                   | Date          |
|----|-----------|------------------------|---------------|
|    | 2,236,519 | Carpenter _____        | Apr. 1, 1941  |
|    | 2,287,467 | Carpenter et al. _____ | June 23, 1942 |

#### OTHER REFERENCES

65 "Alloys of Iron and Silicon" by Greiner, McGraw Hill Book Co., New York, 1933, page 372.